

# UNITED STATES PATENT OFFICE.

ARRIGO TEDESCO, OF TURIN, ITALY, ASSIGNOR TO SOCIETA ANONIMA STABILIMENTI BIAK, OF TURIN, ITALY, A COMPANY OF ITALY.

## METHOD FOR MANUFACTURING ALUMINIUM ALLOYS.

1,350,893.

Specification of Letters Patent. Patented Aug. 24, 1920.

No Drawing.

Application filed July 11, 1919. Serial No. 310,263.

To all whom it may concern:

Be it known that I, ARRIGO TEDESCO, a subject of the King of Italy, and resident of Turin, Italy, have invented certain new and useful Improvements in Methods for Manufacturing Aluminium Alloys, of which the following is a specification.

The present invention has for its object a method for the manufacture of alloys with a high aluminium percentage according to which, instead of alloying directly with the entire aluminium mass the other metals to be comprised in the alloy, an addition alloy is prepared separately, the same containing said metals in the state of an alloy with a reduced amount of aluminium and this addition alloy is thereafter associated in the required percentage with the aluminium bath to produce the final alloy.

Thus the advantage is obtained that the metals to be alloyed with aluminium are in the condition of an alloy with aluminium, this enabling a better mixing of said metals throughout the mass and giving rise to a more homogeneous final alloy having a very fine grain and higher resistance to tensile stresses.

The addition alloy may be alloyed with aluminium to variable percentages that is up to 30% of the final alloy.

It has been found that this method may be carried out with very satisfactory results for producing alloys of aluminium with zinc and copper.

With reference to such a case as an example of this invention, a separate alloy is made containing 66% of zinc, 9% of copper and

25% of aluminium, this alloy being then associated with the aluminium bath to a percentage which may vary up to 30% of the final alloy.

It has been found that the final alloy obtained according to this invention has a resistance to tensile stresses, when cast, up to 35 kg. per sq. mm. and, when rolled, up to 50 kg. per sq. mm.

Obviously percentages of added metals and of aluminium in the addition alloy may vary within wide ranges and the percentage of addition alloy in the final alloy will be accordingly varied so that this latter has the desired characters.

What I claim as my invention and desire to secure by United States Letters Patent is:

1. A method of producing a zinc-copper-aluminum alloy containing a high percentage of aluminum, consisting in preparing, separately from the aluminum bath, an addition alloy comprising about 66% of zinc, 9% of copper and 25% of aluminum; and thereafter associating such alloy, in proportion up to 30% of the final alloy, with the aluminum bath.

2. A method of producing a zinc-copper-aluminum alloy containing a high percentage of aluminum, consisting in preparing, separately from the aluminum bath, an addition alloy comprising about 66% of zinc, 9% of copper and 25% of aluminum; and thereafter associating such alloy with the aluminum bath.

Signed at Turin, Italy, June 12, 1919.

ARRIGO TEDESCO.